

[54] SUBBING MATERIAL FOR STYRENE BASES  
USED IN PHOTOGRAPHIC ELEMENTS

[75] Inventors: Sumitaka Tatsuta; Nobuo Yamamoto;  
Nobuo Tsuji, all of Minami-ashigara,  
Japan

[73] Assignee: Fuji Photo Film Co., Ltd., Minami-  
ashigara, Japan

[21] Appl. No.: 770,147

[22] Filed: Feb. 18, 1977

**Related U.S. Application Data**

[63] Continuation of Ser. No. 561,505, Mar. 24, 1975,  
abandoned, which is a continuation-in-part of Ser. No.  
402,692, Oct. 2, 1973, abandoned.

**Foreign Application Priority Data**

Oct. 2, 1972 [JP] Japan ..... 47-98821

[51] Int. Cl.<sup>2</sup> ..... G03C 1/78  
[52] U.S. Cl. ..... 96/87 A; 96/29 R;

96/87 R; 427/40; 427/407 C

[58] Field of Search ..... 427/40, 407; 96/87 R,  
96/29 R, 87 A

[56]

**References Cited**

**U.S. PATENT DOCUMENTS**

|           |         |                      |          |
|-----------|---------|----------------------|----------|
| 2,306,071 | 12/1942 | McNally et al. ....  | 260/78   |
| 3,007,901 | 11/1961 | Minsk .....          | 260/78.3 |
| 3,232,756 | 2/1966  | Yakel et al. ....    | 96/87 R  |
| 3,454,424 | 7/1969  | Schneider .....      | 96/87 R  |
| 3,492,122 | 1/1970  | Takenaka et al. .... | 96/87 R  |
| 3,527,605 | 9/1970  | Fisch et al. ....    | 96/87 R  |
| 3,645,740 | 2/1972  | Nishio et al. ....   | 96/87 R  |
| 3,679,455 | 7/1972  | Kasugai et al. ....  | 96/87 R  |
| 3,770,443 | 11/1973 | Osuda et al. ....    | 96/87 R  |
| 3,811,913 | 5/1974  | Kasugai et al. ....  | 96/87 R  |
| 3,867,167 | 2/1975  | Tatauto et al. ....  | 96/87 R  |

*Primary Examiner*—Jack P. Brammer

*Attorney, Agent, or Firm*—Sughrue, Rothwell, Mion,  
Zinn and Macpeak

[57]

**ABSTRACT**

A photographic material comprising (I) a styrene-based polymer support having thereon a subbing layer which comprises a partial or complete reaction product of (a) a copolymer of styrene or vinyl acetate with maleic anhydride with (b) water or a hydroxy compound such as alcohol and (II) a photographic layer comprising a hydrophilic resin binder bearing on the subbing layer, wherein a compound containing two or more epoxy groups per molecule is contained in the subbing layer or in both of the subbing layer and the photographic layer.

20 Claims, No Drawings

**SUBBING MATERIAL FOR STYRENE BASES  
USED IN PHOTOGRAPHIC ELEMENTS**

**CROSS-REFERENCE TO RELATED APPLICATION**

This application is a continuation application of Ser. No. 561,505, filed Mar. 24, 1975 now abandoned, in turn a Continuation-In-Part of U.S. Application Ser. No. 402,692 filed Oct. 2, 1973, in the name of Sumitaka Tatsuta et al, entitled "Photographic Material", now

**BACKGROUND OF THE INVENTION**

**1. Field of the Invention**

This invention relates to a photographic material comprising a film support of a polymer comprising substantially a polymer of styrene and having thereon a subbing layer which has strong adhesivity to a photographic layer comprising a hydrophilic resin binder, such as light-sensitive layers or image-receiving layers as are used in conventional photography.

**2. Description of the Prior Art**

Generally a polymeric film consisting mainly of styrene is a desirable material for a photographic support because of its excellent transparency, physical strength, dimensional stability and strength. However, such a support has a very hydrophobic surface, as is apparent from the molecular structure, so some pretreatment such as undercoating is necessary to provide a photographic layer consisting of a hydrophilic resin binder on the support with strong adhesion such that the photographic layer does not separate from the support during processing and using.

As a method of undercoating a photographic support consisting substantially of a styrene polymer, it is known to use homopolymers or copolymers of acrylic acid esters, methacrylic acid esters, acrylic acid, methacrylic acid and acrylamide, or copolymers thereof with styrene.

However, a one layer coating of the above-mentioned (co)polymers on the support is insufficient to obtain effective results and, therefore, complicated multi-layer undercoating has been carried out in practice. For example, undercoating using a three layer structure is most commonly conducted wherein a polymer layer of the above-mentioned acrylic type is provided as a first layer, a nitrocellulose layer is used as a second layer and further a dispersion of gelatin in an organic solvent is employed as a third layer. Such multi-layer undercoating is most undesirable because of the required complicated processing, the increase in the production cost and the deterioration in the stability of a product. Furthermore, this method is dangerous because it is necessary to use a very flammable nitrocellulose resin.

U.S. Pat. No. 3,072,482 Beeber et al discloses vinyl methyl ether-maleic anhydride polymer used in a small amount in a subbing layer as a supplementary component of the subbing layer where a gelatin subbing solution (cf. Col. 2) is necessary.

U.S. Pat. No. 3,645,740 Nishio et al and U.S. Pat. No. 3,770,443 Osada et al disclose photographic elements which contain epoxy compounds useful in the present invention.

U.S. Pat. No. 3,527,605 Fisch et al discloses epoxidized materials useful in a subbing layer.

As a result of research on suitable undercoating materials for the purpose of overcoming the above-described disadvantages, it has been found that a complete or partial reaction product of a copolymer of styrene or

vinyl acetate with maleic anhydride with water or a hydroxy compound represented by the general formula  $R_1-OH$ , wherein  $R_1$  is a monovalent hydrocarbon group having 1 to 12 carbon atoms or monovalent organic group having 2 to 12 carbon atoms and consisting of at least two hydrocarbon fragments and at least one ether linkage between said hydrocarbon fragments ( $R_1$  does not represent cyclic ether linkage), preferably an alkyl group, is very effective for the adhesion of a hydrophilic photographic layer to a support of a polymer consisting predominantly of styrene. The above-described copolymer has in its polymeric structure, at least partially, recurring units having the formula:



in which  $R_3$  is a hydrogen atom or a group described above for  $R_1$  and  $R_2$  is a phenyl group (when the copolymer is a styrene copolymer) or a  $-\text{OCOCH}_3$  group (when the copolymer is a vinyl acetate copolymer).

When a support of a polymer consisting mainly of styrene is undercoated with the above-described copolymer, the adhesiveness of a hydrophilic photographic layer to this support is markedly increased, but the undercoated layer must be quite thick, i.e., a thickness of more than several microns. Accordingly, coating and surface difficulties often take place. Furthermore, the adhesive strength is not quite as sufficient as desired, in particular, when wetted in a strongly alkaline developer.

**SUMMARY OF THE INVENTION**

We have now surprisingly found, as a result of our studies to overcome the above-described two disadvantages, an undercoating material capable of imparting an excellent adhesive strength and yet a very thin layer, both at the time of drying as well as on wetting, by the joint use, with the above-mentioned copolymer, of an epoxy compound.

That is to say, in accordance with the present invention, a photographic material is provided having an undercoating layer containing a complete or partial reaction product of a copolymer of styrene or vinyl acetate and maleic anhydride with water or a hydroxy compound represented by the general formula  $R_1-OH$ , wherein  $R_1$  is a hydrogen when the compound is water, a monovalent hydrocarbon group having 1 to 12 carbon atoms or monovalent organic group having 2 to 12 carbon atoms and consisting of at least two hydrocarbon fragments and at least one ether linkage between said hydrocarbon fragments ( $R_1$  does not represent cyclic ether linkage) when the compound is a hydroxy compound, and a compound containing two or more epoxy groups per molecule on a support member of a polymer consisting predominantly of styrene.

At least 30 mol %, and preferably more than 60 mol %, of the units of maleic anhydride in the copolymer should react with the hydroxy compound or with water.

The percentage of maleic anhydride in the copolymer is from 40 to 50% by weight, preferably about 50% by weight, based on copolymer weight.

#### DETAILED DESCRIPTION OF THE INVENTION

As the monovalent hydrocarbon group there are an alkyl group, a phenyl group, and a phenylalkyl group, and as the monovalent organic group which contains at least one ether linkage in the group there are an alkoxy-alkyl group, an alkoxyalkoxyalkyl group and a phenoxyalkyl group.

As described above, water or a hydroxy compound of the formula  $R_1-OH$  such as methanol, ethanol, propanol, isopropanol, butanol, sec-butanol, amylalcohol, sec-amylalcohol, isoamylalcohol, 2-ethylhexylalcohol, octanol, nonanol, decanol, t-octanol, dodecanol, phe-

noxyethanol, methoxyethanol, butoxyethanol, acetoxethanol,  $\beta$ -methoxyethoxyethanol, phenylpropanol, and the like, is employed in preparing the copolymer used in this invention. Mixtures of such hydroxy compounds can be used, if desired.

A support member having the undercoating layer according to the present invention favorably compares to one having an undercoating layer consisting only of the above-described copolymer with respect to the 10 adhesiveness to a hydrophilic photographic layer.

As the epoxy compound of the invention, any poly-functional epoxy compound having at least two epoxy groups in the molecule can be used. The epoxy compound will generally have a molecular weight less than 15 about 20,000 preferably less than 1,000. Typical of such epoxy compounds are the following compounds:

#### Typical Epoxy Compounds



-continued

## Typical Epoxy Compounds



-continued

## Typical Epoxy Compounds



-continued



(33) a polymer of glycidyl acrylate or glycidyl methacrylate, or a copolymer thereof with polymerizable ethylenically unsaturated compounds such as glycidyl acrylate, glycidyl methacrylate, ethylene, styrene, vinyl chloride, vinylidene chloride, acrylic acid, an acrylic ester, methacrylic acid, a methacrylic ester, acrylonitrile and an acrylic amide.

(34) a polymer of compound 12 (usually a polymer having a molecular weight lower than 1,000 is 40 used).

It shall be specifically understood that the exact epoxy compound used is not critical so long as it is polyfunctional and contains at least two epoxy groups.

These epoxy compounds can be prepared using known methods, for example, by treating a compound having an active hydrogen containing group, such as a hydroxyl, carboxyl, amino, imino or amide group with a halohydrin, such as epichlorohydrin, epibromohydrin, methyl-epichlorohydrin, or methyl-epibromohydrin, by 45 treating a compound containing an active halogen such as the acid halides, for example, the sulfonic acid halides, with glycidol, or by subjecting an ethylenically unsaturated compound to an oxidation treatment. These polyfunctional epoxy compounds used in the present 50 invention and their preparation are disclosed in "Epoxy Resins Their Application and Technology", McGraw Hill Book Co., Inc., New York (1957), pages 15-21, "Epoxy Resin Technology", Interscience Publishers, New York (1968), pages 2-14, U.S. Pat. No. 3,562,275, U.S. Pat. No. 3,620,983 and Swiss Pat. No. 471,811. Some of these compounds are commercially available, for example, as Araldite-6005 and Araldite-6010 from Ciba Co., Inc. and as Epon-820 and Epon-828 from Shell Chemical Co. Epoxy compounds (3), (6), (7), (12) and (23) are particularly preferred.

Mixtures of such epoxy compounds can be used, if desired.

The above-described epoxy compound used in the invention is mixed with the copolymer containing maleic acid ester units and the resulting mixture is coated onto a support of a polymer consisting predominantly of styrene, followed by a further coating of a hydrophilic photographic layer.

It is not completely clear why the undercoated layer according to the invention strengthens the adhesion between the support and the hydrophilic photographic layer. However, the wetting adhesive strength in various photographic processing baths is markedly increased by the practice of the invention. This is possibly due to the formation of an insoluble network structure by the self bridging reaction of the polyfunctional epoxy compound in the undercoated layer end by the bridging reaction of the polyfunctional epoxy compound with the maleic acid ester unit-containing copolymer having a number of carboxyl groups as side chains serves to suppress stripping and breaking of the support/undercoated layer/hydrophilic photographic layer at the layer boundary and to prevent the undercoated layer from dissolving out. Moreover, it is assumed that a polyfunctional epoxy compound used in the invention and its self bridging product fulfill a plasticizing effect on the maleic acid ester unit-containing copolymer, suppress generation of internal stresses in the undercoated layer containing the copolymer and thus prevent the aggregation and breakage thereof. This effect not only provides the ability to use a much thinner undercoating than can be used when the undercoated layer consists only of the copolymer but also increase the adhesive strength at the time of drying.

The present invention will now be illustrated in greater detail.

In the present invention, the term "support composed of a styrene-base polymer" is used herein to mean a support which is fabricated into a film from a homopolymer of styrene, a homopolymer of a substituted styrene which is exemplified by  $\alpha$ -methyl styrene, chlorostyrene, vinyl toluene and the like, or copolymers of styrene with a copolymerizable comonomer such as ethylene, butadiene, isoprene, vinyl chloride, vinylidene chloride, vinyl acetate, vinyl propionate, acrylic or methacrylic acid esters (for example, the methyl, ethyl, butyl, ethylhexyl, methoxyethyl cyclohexyl, lauryl ester, etc.), acrylic acid or methacrylic acid amides (for example, acrylamide, methacrylamide, diacetone acrylamide), vinyl methyl ether, vinyl butyl ether, vinyl chloroethyl ether, etc., or mixtures of such materials, which are exemplified by a styrene/butadiene copolymer, a styrene/acrylonitrile copolymer, etc. The styrene content in the polymer or copolymer can range from about 10 to 100 wt.%, based on the weight of the polymers in the support. Basically any of these materials which will form a film can be employed and accordingly the molecular weights are not limiting. Generally, molecular weights ranging from about 5,000 to about 2,000,000, preferably 80,000 to about 500,000, are employed from a practical standpoint. Hereinafter, the term "support" means a support composed of the styrene-base polymer as described above, unless otherwise indicated.

The support can be a transparent film or can be a film having a filler, such as  $TiO_2$ ,  $CaCO_3$ ,  $Al_2O_3$ ,  $ZnO$ , carbon black, etc., incorporated therein at a filler content of from about 1 to 10 wt.%, preferably 2 to 4 wt.% based on the weight of the polymer(s). Additives such

as dyes, fluorescent whitening agents, antistatic agents, etc., can be incorporated in the support in conventional amounts. The surfaces of the support can be roughened as in a synthetic paper, as described, for example, in U.S. Pat. No. 3,723,159. The presence or absence of these additives or modifiers gives rise to no adverse influences on the effects of the present invention since the support is mainly composed of styrene.

The surface of the support described above adheres extremely strongly to a photographic layer comprising a hydrophilic resin binder. The term thus photographic layer comprising a hydrophilic resin binder" includes a hydrophilic colloid layer containing silver halide, silver iodobromide, silver iodochloride, silver chloride, silver chlorobromide, silver bromide, etc., as in a black and white film, a color film or a printing paper, a hydrophilic colloid layer containing physical developing nuclei such as silver sulfide, as in a receiving layer used in diffusion transfer photography, a photographically conventional backing layer which is coated on the back of the support for the purpose of curl preventing, antihalation, etc., and so on. The hydrophilic resin which is most commonly used as a photographic layer is gelatin and other examples are graft-gelatin, acylated gelatin, etc., and natural or synthetic hydrophilic resins which are exemplified by casein, agarose, polyvinyl alcohol, polyvinyl pyrrolidone, vinyl pyrrolidone and a vinyl alcohol copolymer with another monomer such as acrylic acid, methacrylic acid, or the amide or ester thereof such as the methyl, ethyl, hydroxypropyl, methoxyethyl, hydroxyethyl, ethoxybutyl esters, vinyl methyl ether, vinyl propionate, styrene maleic anhydride, and the like, etc. The support subbed with the material in accordance with the present invention can adhere extremely strongly to photographic layers comprising any of the hydrophilic resins described above. The adhesion thus obtained does not deteriorate after the passage of time both for a film prior to exposure, i.e., as initially prepared, and after development processing.

The undercoating method according to the present invention consists in preparing a solution of the foregoing copolymer and epoxy compound in water or an organic solvent, applying the solution to a support and drying. Illustrative solvents for the foregoing copolymer are alcohols such as methanol, ethanol and propanol, ketones such as acetone and methyl ethyl ketone, and halogenated hydrocarbons such as methylene chloride and trichlene. The epoxy compound is soluble in acetone, dimethylformamide and methanol, and mixtures with other solvents.

In the photographic material of the invention, the undercoating can be carried out using any solvent, but, in general, alcohols being a non-solvent for the support, in particular, methanol, are preferably used as a solvent, since ketones and halogenated hydrocarbons swell or dissolve the support consisting predominantly of styrene. The support is very stable toward alcohols and methanol is less expensive than other solvents. Of course, a suitable amount, for example, less than 50% by weight based on the weight of non-solvent of the support of another solvent (ketones such as acetone, methyl ethyl ketone, methylisobutyl ketone, etc., halogenated hydrocarbons such as trichloromethylene, dichloroethylene, methylene dichloride, etc.) can be used if desired.

The amounts of the copolymer and epoxy compound used are not particularly limited, but the former is pref-

erably used in an amount of 0.01 to 5 g or less, preferably 0.1 to 2 g, per 1 m<sup>2</sup> of the support, while the latter is generally used in a proportion of 10 to 500, preferably 50 to 200, percent by weight based on the weight of the copolymer used. The copolymer generally has a molecular weight ranging from about 8,000 to about 1,000,000 with an intrinsic viscosity  $[\eta]$  of about 0.05 to about 1.0 measured in methyl alcohol at 30° C.

In the undercoating of the invention, only a mixture of the foregoing copolymer and epoxy compound need be coated onto a support, but the joint use of gelatin therewith provides better results. Where gelatin is used, up to about 300 wt.%, preferably about 50 to 150 wt.%, gelatin to the copolymer can be employed. For example, when the above-described copolymer and epoxy compound are dissolved in an organic solvent in a conventional manner followed by a dispersion of gelatin therein and the resulting solution is used as an undercoating solution, a very fine surface and excellent adhesion can be obtained. Another method comprises applying only the mixed solution of the copolymer and the epoxy compound to a support, drying and then applying a dispersion of gelatin in an organic solvent. In a further embodiment of the invention, an undercoated layer of the copolymer is first provided on a support and then a photographic layer containing the epoxy compound is coated (see Example 6), whereby the epoxy compound is diffused into the undercoated layer. The amount of epoxy compound in the undercoated layer, which is diffused from the photographic layer, preferably is in the range disclosed above, i.e., 10 to 500, preferably, 50 to 200% by weight, based on the weight of copolymer used. The amount of diffusion depends on the thickness of the photographic layer, but usually in the photographic layer the epoxy compound is used in an amount of 20 to 1,000% based on the weight of the copolymer used. The thickness of the photographic layer containing an epoxy compound may be optionally selected, but usually it is in a range of 0.1 to 60 microns. The thickness does not effect the adhesivity in the present invention. The epoxy compound may be added into the photographic layer composition as a solution of a solvent either compatible or incompatible with water. In the latter case the epoxy compound is emulsified mechanically or by using an emulsifier. With any method, the advantages of the present invention are obtained.

The concentration of the undercoating solution is not particularly limited, but can be optionally determined depending on the coating means. In the case of an immersion coating method or a reverse roll coating method, for example, the viscosity can be adjusted with a solvent to about 1 cps, while in the case of a gravure coating method, it can be about 10 cps. This undercoating solution is very stable in any concentration. Drying of the undercoating solution after being coated can be conducted at a suitable temperature, preferably room temperature (e.g., about 20° to 30° C) to about 100° C.

With respect to drying, the prior art undercoating methods are considerably restricted regarding this point. That is, the drying must be carried out within a limited temperature range in order to obtain sufficient adhesion and, therefore, slight fluctuations of temperature often cause adhesion difficulties. Where the undercoating material according to the invention is used, on the contrary, a constant and good adhesion can always be obtained over a wide drying temperature range from

room temperature to the softening temperature of the support itself, i.e., about 100° C. This difference is probably due to the fact that, with prior art undercoating, an etching solvent for the support must be used so as to obtain adhesion of the undercoated layer to the support through the anchor effect of the etching agent, while in the method of the invention, adhesion can be obtained due only to the chemical affinity of the undercoated layer and support without the need for any etching agents. In general, the etching power of the solvent used depends on the temperature and adhesion due to the anchor effect is greatly affected by temperature during coating or drying, while adhesion due to chemical affinity is not so affected by temperature.

The proper drying time in the present invention can be determined easily by experimentations. It depends on the solvent and the concentration of the undercoating solution. The drying time does not affect the adhesivity practically.

If the epoxy compound is contained in a photographic layer, the drying time can be determined as described above but the drying temperature should be determined carefully to prevent from deteriorating characteristics of the photographic layer by heating.

It is a great industrial advantage that the undercoating of the present invention can be achieved over a broad temperature range. In order to increase the advantages of the invention, surface activating treatments such as an electric discharge such as a corona discharge as described in U.S. Pat. Nos. 2,864,755 and 2,864,756 and electroless discharge as described in British Pat. No. 1,294,116, an ozone oxidation, an ultraviolet radiation, a flame treatment as described in U.S. Pat. No. 3,072,483, a chromate-mixed acid treatment (before coating) are very effective before or after coating of the above described undercoating solution. This activating treatment can be carried out using conventionally known techniques and apparatus. In the case of electric discharge, for example, there are methods wherein a support is exposed to DG or AG corona atmosphere produced by applying a voltage between a pair of electrodes and wherein an electric field of high frequency is generated under reduced pressure in a discharge bulb and a support is treated with molecules excited thereby, which is called "non-electrode discharge treatment." Ultraviolet irradiation can be carried out using a high voltage mercury lamp.

Some polar groups are formed on the surface of polystyrene, which is naturally hydrophobic, by these treatments and the surface is thus made hydrophilic. Consequently, the affinity with the polar groups in the copolymer contained in the undercoated layer is increased.

In the photographic material undercoated according to the invention, as described above, the support comprising predominantly of polystyrene adheres strongly to a photographic layer comprising the hydrophilic binder at the time of drying as well as wetting, and the thus resulting adhesion is not deteriorated by the passage of time either in the state of the film as initially prepared or after development.

In this specification, the disclosure is directed particularly to photography, but, it will be apparent to those skilled in the art that the present invention can be applied to any field where adhesion between a polymeric molding comprising predominantly polystyrene and a hydrophilic resin is involved.

The following examples are to illustrate the invention in greater detail but these examples are not to be interpreted as limiting the invention. In the examples, unless otherwise indicated, all parts and percents are by weight.

In the examples, adhesiveness tests were carried out according to the procedures described below:

#### 1. Test method of adhesiveness of dry film

A photographic layer to be tested was notched 6 times at intervals of 5 mm, respectively, in length and width to form twenty-five squares, an adhesive tape such as a polyester tape was adhered thereto and stripped quickly at a direction of 180°. Based on the number of the stripped squares on the photographic layer, the adhesiveness was assessed using the five grades described as follows:

| Grade | Number of Stripped Squares |
|-------|----------------------------|
| A     | 0 - 5                      |
| B     | 6 - 10                     |
| C     | 11 - 15                    |
| D     | 16 - 20                    |
| E     | 21 - 25                    |

#### 2. Test method of adhesiveness of wet film

A film was notched using an iron pen to give a mark *x* in each of the development solutions and rubbed strongly twenty times using finger tip. Based on the maximum width stripped along the *x* line, the adhesive force was assessed using the five grades described as follows:

| Grade | Maximum Stripped Width |
|-------|------------------------|
| A     | 0 - 0.9 m/m            |
| B     | 1.0 - 2.9 m/m          |
| C     | 3.0 - 5.0 m/m          |
| D     | No Resistance          |
| E     | Spontaneous Stripping  |

In all Examples coating was carried out at room temperature (about 25° C).

#### EXAMPLE 1

200 g of a copolymer of maleic anhydride and styrene (molar ratio 1:1) (limiting viscosity  $[\eta] = 0.615$  measured at 30° C in ethyl acetate) was added to 800 g of 50 methanol, heated with agitation and reacted for 8 hours with refluxing (about 85° - 95° C). After the reaction, the infrared spectrum of the product showed that the absorption at 1850  $\text{cm}^{-1}$  (corresponding to the absorption of the acid anhydride C=O) disappeared. The acid 55 number was  $3.9 \times 10^{-3}$  equivalents/g. After the reaction, the polymer concentration was adjusted to 20% by weight (methanol solution).

To 5 ml of this solution were added 85 ml of methanol and 10 ml of trichloroethylene and then 1.1 g of the 60 epoxy compound represented by Epoxy Compound (3), hereinbefore described, was added thereto to prepare an undercoating solution.

On the other hand, a biaxially stretched polystyrene support was subjected to a corona discharge treatment at a distance of 2 mm between the polystyrene support and the electrode and at a support speed of 2 m/min and a discharge output of 200 W. The thus treated support was coated at a coating rate of 5 m/min with the above-

described undercoating solution using immersion coating and dried at 80° C. The undercoated polystyrene support was coated with a gelatino-silver halide color photographic emulsion having the following composition per 1 m<sup>2</sup>:

|                                                                                             |        |
|---------------------------------------------------------------------------------------------|--------|
| Silver Chlorobromide                                                                        | 3.0 g  |
| Gelatin                                                                                     | 3.5 g  |
| Benzoylaceto-2-chloro-5-dodecyloxy-carbonyl anilide (yellow coupler) emulsified dispersion* | 14.0 g |
| Triethylene Phosphamide (3% acetone solution)                                               | 3.0 ml |
| Polyvinylpyrrolidone (mol wt. approx. 360,000)                                              | 0.7 g  |

The adhesive strength between the emulsion layer and the support in the resulting photographic material was a Grade A before, during and after development.

For comparison, a polystyrene support was subjected to a corona discharge treatment under the same conditions as described above, coated with the same undercoating solution as described above, but not containing the epoxy compound, and then coated with the same photographic emulsion. The adhesive strength of the resulting photographic material was Grade D before and after development, and Grade C during development.

For further comparison, vinyl methyl ether was used instead of styrene in the aforesaid experiment, in combination with the epoxy compound. The adhesive strength of the resulting photographic material was Grade E before and after development and during development.

#### EXAMPLE 2

4 g of gelatin was swollen in 10 g of water and then mixed with 1.4 g of salicylic acid and 500 ml of methanol with stirring to prepare a dispersion of gelatin in methanol. To 100 ml of this dispersion were added 3.8 ml of the 20% copolymer solution of Example 1 and then 2.7 g of the epoxy compound represented by Epoxy Compound (23) to prepare an undercoating solution.

On the other hand, a biaxially stretched high impact polystyrene support containing 10% by weight of titanium dioxide was subjected to a corona discharge treatment under the same conditions as that of Example 1 and then coated with the above described undercoating solution at a coating rate of 5 m/min by immersion coating, followed by drying at room temperature. The thus undercoated support was coated with a black-and-white gelatino-silver halide photographic emulsion having the following composition per 1 m<sup>2</sup> of the support:

|                         |        |
|-------------------------|--------|
| Silver Chlorobromide    | 3.5 g  |
| Gelatin                 | 13.0 g |
| Formaldehyde (hardener) | 0.1 g  |
| Saponin (wetting agent) | 0.03 g |

The adhesive strength between the emulsion layer and support of the resulting photographic material was a Grade A in both cases of a wet film during development and a dry film after development.

For comparison, the same support was undercoated with the same undercoating solution as described above but not containing the epoxy compound and then coated with the same photographic emulsion as above. The adhesive strength of the resulting photographic

material was Grade C in both the dry state and the wet state.

#### EXAMPLE 3

5 In the undercoating composition of Example 2, 3 g of the epoxy compound represented by Epoxy Compound (6) was added in place of the Epoxy Compound (23) to prepare an undercoating solution. A commercially available polystyrene synthetic paper (QU-33) produced by Nihon Goseishi Co., Ltd. was coated with the undercoating solution, dried at 70° C and then coated with a coating solution for forming an image receiving layer of an image receiving material used in silver salt diffusion transfer photography, having the following composition per 1 m<sup>2</sup> of film:

|                                    |         |
|------------------------------------|---------|
| Gelatin                            | 3 g     |
| Silver Sulfide (developing nuclei) | 0.001 g |
| Phenylmercaptotetrazole (toner)    | 0.01 g  |
| Saponin (wetting agent)            | 0.02 g  |

The adhesive strength of this image receiving material was Grade A in both the dry state and the wet state.

25 For comparison, a similar test was carried out on the same photographic material but using an undercoating solution which did not contain any epoxy compound. The adhesive strength was Grade B in the dry state and Grade C in the wet state.

#### EXAMPLE 4

20 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 92

thereto to extract the N-hexyl alcohol from the solid product. This procedure was repeated two or three times and, after removing the solvent, the polymeric solid was dried. The acid number was  $2.51 \times 10^{-3}$  equivalents/g and the ring opening ratio was about 70%. 1 g of the resulting polymer was dissolved in 100 ml of the dispersion of gelatin in methanol as used in Example 2 and 1.2 g of the epoxy compound represented by Epoxy Compound (3) was added to this solution to prepare an undercoating solution. On the other hand, a biaxially elongated high impact polystyrene support containing 8% by weight of titanium dioxide was subjected to a corona discharge treatment under the same conditions as those of Example 1, coated with the same undercoating solution as described above followed by drying, and then coated with the same black-and-white silver halide photographic emulsion as that of Example 2. The adhesive strength between the support and the photographic layer was Grade A in both the dry state and the wet state.

For comparison, a similar test was carried out on the same photographic material but using an undercoating solution which did not contain an epoxy compound. The adhesive strength was Grade C in both the dry state and the wet state.

Example 6 below exemplifies preparing a photographic material in which an epoxy compound is in the emulsion layer, while Example 7 exemplifies preparing a photographic material in which a copolymer of an epoxy compound is contained in an undercoating layer.

#### EXAMPLE 6

An undercoating solution as in Example 1 was prepared except without adding an epoxy compound.

A biaxially stretched polystyrene support was subjected to corona discharge treatment under the same condition as in Example 1 and was then coated with the above described undercoating solution at a coating rate of 5 m/min by a conventional immersion coating technique, followed by drying at 80° C. The thus obtained undercoated support was coated with a black-and-white gelatin-silver halide photographic emulsion having the following composition per 1 m<sup>2</sup> of the support and dried:

|                      |        |
|----------------------|--------|
| Silver Chlorobromide | 3.5 g  |
| Gelatin              | 13.0 g |
| Epoxy Compound (3)   | 20.0 g |
| Water                | 150 g  |
| Saponin              | 0.03g  |

The adhesive strength between the emulsion layer and the support in the resulting photographic material was Grade A in all cases for the dry film both before and after development, and was Grade A for a wet film during development.

#### EXAMPLE 7

4 g of gelatin was swollen by 10 g of water, and then 1.4 g of salicyclic acid and 500 ml of methanol were added with agitation into the swollen gelatin to prepare a gelatin dispersion in methanol.

To 100 ml of the dispersion thus obtained 3.8 ml of 20% by weight of the copolymer solution described in Example 1 was added, and then 10 g of a 10% by weight solution of acrylic acid-glycidyl acrylate copolymer (molar ratio 7:3: softening point 80° C) in dioxane-tet-

rahydrofuran (1:1 by weight) was added thereto to yield an undercoating solution.

A biaxially stretched high impact polystyrene support was subjected to corona discharge treatment under the same conditions as in Example 1 and then coated with the above-described undercoating solution at a coating rate of 5 m/min by a conventional immersion coating technique, followed by drying at 90° C for 10 minutes.

The thus obtained undercoated support was coated with a gelatino-silver halide color photographic emulsion having the same composition as in Example 1.

The adhesive strength between the emulsion layer and the support in the resulting photographic material was Grade A in all cases for the dry film before and after development, and was Grade A for the wet film during development.

While the invention has been described in detail and with reference to specific embodiments thereof, it will be apparent to one skilled in the art that various changes and modifications can be made therein without departing from the spirit and scope thereof.

What is claimed is:

1. A method for manufacturing a photographic material which comprises coating a subbing composition in layer form on a styrene-based polymer support, said composition consisting essentially of 5g or less per m<sup>2</sup> of said support of a complete or partial reaction product of materials consisting essentially of (a) a copolymer of styrene or vinyl acetate with maleic anhydride which contains 40-50% by weight of maleic anhydride with (b) water or a hydroxy compound represented by the general formula R<sub>1</sub>-OH wherein R<sub>1</sub> is a monovalent hydrocarbon group having 1 to 12 carbon atoms or monovalent organic group having 2-12 carbon atoms and consisting of at least two hydrocarbon fragments and at least one ether linkage between said hydrocarbon fragments, at least 30% of the maleic anhydride units of said copolymer being reacted with the water or the hydroxy compound thereby obtaining a reaction product consisting essentially of the following recurring units:



in which R<sub>3</sub> is a hydrogen atom or a group defined by R<sub>1</sub>, R<sub>2</sub> is a phenyl group or a -OCOCH<sub>3</sub> group and the amount of the maleic anhydride unit in said copolymer may be zero, and coating a hydrophilic photographic composition containing a hydrophilic resin binder in layer form on the subbing layer, where the resulting hydrophilic photographic composition layer is selected from the group consisting of (1) a layer containing silver halide, (2) a layer containing physical developing nuclei to serve as a receiving layer in diffusion transfer photography, a hydrophilic photographic curl preventing backing layer or a hydrophilic photographic anti-halation backing layer, where a compound containing at least two epoxy groups per molecule is contained in a proportion of from 10 to 500% by weight based on the weight of said copolymer in at least one of the subbing

composition or the hydrophilic photographic composition.

2. The method of claim 1 in which said compound containing two or more epoxy groups per molecule is in the subbing composition.

3. The method of claim 1 in which said compound containing two or more epoxy groups per molecule is in the hydrophilic photographic composition.

4. The method of claim 1 in which said compound containing epoxy groups has a molecular weight less than about 20,000.

5. The method of claim 1 in which said compound containing epoxy groups has a molecular weight less than 1,000.

6. The method of claim 1 wherein said compound containing two or more epoxy groups is selected from the group consisting of:



7. The method of claim 1 wherein said subbing composition additionally contains gelatin.

8. The method of claim 1 wherein said complete or partial reaction product of said copolymer has a molecular weight ranging from about 8,000 to about 1,000,000.

9. The method of claim 1 wherein R<sub>1</sub> is an alkyl group, a phenyl group, a phenylalkyl group, an alkoxy-alkyl group, an alkoxyalkoxyalkyl group, or a phenoxyalkyl group.

10. The method of claim 1 wherein said hydroxy compound is an alcohol and said R<sub>1</sub> is selected from the group consisting of methyl, ethyl, propyl, butyl and lauryl.

11. The method of claim 1 wherein said subbing composition is coated on said support after a surface pretreatment of said support.

12. The method of claim 11 wherein said surface pretreatment is by a corona discharge treatment, an ozone oxidation treatment, an ultraviolet irradiation treatment, a flame treatment, an electroless discharge treatment, or a low pressure electric discharge treatment.

13. The method of claim 1, wherein hydrophilic hydrophilic composition is in the form of an emulsion or dispersion.

14. The method of claim 1, wherein said hydrophilic photographic composition is in the form of a solution.

15. The method of claim 1, wherein said hydrophilic composition contains silver halide.

16. The method of claim 1, wherein said hydrophilic composition contains physical development nuclei.

17. The method of claim 1, wherein said hydrophilic resin binder in said hydrophilic photographic composition comprises gelatin.

18. The method of claim 1, wherein said hydrophilic resin binder in said hydrophilic photographic composition consists of gelatin.

19. The method of claim 1, wherein said copolymer consists of a copolymer of styrene and maleic anhydride.

20. The method of claim 1, wherein said copolymer consists of a copolymer of vinyl acetate and maleic anhydride.

\* \* \* \* \*